

Jan. 2, 1951

J. SPENCER

2,536,323

POLYVINYL CHLORIDE PRINTING ROLLER

Filed March 18, 1947



Fig. 1



Fig. 2

INVENTOR  
J. SPENCER  
By: Fetherstonhaugh & C.  
ATT'YS

## UNITED STATES PATENT OFFICE

2,536,323

## POLYVINYL CHLORIDE PRINTING ROLLER

James Spencer, Toronto, Ontario, Canada, assignor to Perma-Flex Industries Limited, Toronto, Ontario, Canada, an incorporated company of Ontario

Application March 18, 1947, Serial No. 735,297

3 Claims. (Cl. 154—43)

**1**  
This invention relates to a material for making printing rollers and plates and a method for making the same.

Hitherto, printing rollers have generally been made from a composition of glycerine and animal glue which is suitably processed and cast to give the surface characteristics necessary for the purpose. Various attempts have been made to use synthetic materials for the production of such rollers but up until the present these have been unsuccessful. The chief drawbacks to using the animal glue-glycerine roller, which is in all other respects highly satisfactory, are that it is water soluble and, therefore, cannot be used with inks which have water as a component and, further, the glycerine rollers will melt at temperatures above 100° F. and, consequently, are unsuitable for high speed rollers where temperatures are often in excess of this figure. Rollers of this type are further subject to the disadvantage that their dimensions alter under different conditions of humidity.

Accordingly, it is the object of the present invention to provide a printing roller which can be used with inks containing a wide range of materials including water.

It is another object of the invention to provide a printing roller which may be used at temperatures up to 250° to 300° F. without loss of efficiency.

It is a further object of this invention to provide a simple process for making such rollers.

Figure 1 is a diagrammatic sectional side view of a mold suitable for purposes of the invention.

Figure 2 is a partly cut-away perspective view of a finished roller.

Figure 3 is a plan view of one of the spacer elements used to position the metal core within the mold shown in Figure 1.

Referring now more specifically to the drawings, Figure 1 shows generally the arrangement of the mold which is generally completely housed within a temperature control oven at a temperature slightly in excess of the temperature of the plastic being poured. The mold consists of a hollow cylinder 10 within which are annular ribs 11 which are discontinuous to provide for passage and support of spacer element 12 which is used to support the metallic roller core 13. The cylinder 10 is completely housed within a water jacket 14 provided with inlet 15 and outlet 16 and a gate tube 17 communicates with the bottom part 18 of the cylinder 11 to introduce the melted plastic thereto. The molding operation is as follows:

**2**  
The complete molding apparatus is brought up to a temperature slightly in excess of the melt in a temperature control oven and the melt is introduced in the funnel 19 at the end of the gate tube 17. The melt feeds down into the bottom of the mold and gradually follows it to a point above the upper spacer member 12. This operation is carried out fairly slowly to obviate the inclusion of air bubbles within the body of the plastic. As soon as the mold is full, cooling water is introduced into the water jacket through inlet 16 and the mold is cooled rapidly and evenly to room temperature and the completed roller 20 is removed and trimmed to size.

Suitable proportions of ingredients are best illustrated by reference to the following examples:

*Example I*

|                       | Parts by weight |
|-----------------------|-----------------|
| 20 Polyvinyl chloride | 100             |
| Di-octyl phthalate    | 130             |
| Ester gum             | 1               |
| Burnt sienna          | 5               |

**25** The above composition produces a rubbery substance suitable for high speed rollers and with only a slight amount of tack on the surface.

*Example II*

|    |                    |     |
|----|--------------------|-----|
| 30 | Polyvinyl chloride | 100 |
|    | Plasticiser        | 130 |
|    | Ester gum          | 5   |
|    | Burnt sienna       | 5   |

**35** The substance produced by the above proportions of ingredients is very much the same as that in the above example with the exception that the above composition surface is considerably more tacky.

*Example III*

|    |                    |     |
|----|--------------------|-----|
| 40 | Polyvinyl chloride | 100 |
|    | Di-octyl phthalate | 200 |
|    | Ester gum          | 1   |

**45** A slightly softer composition with a surface tack suitable for normal printing purposes.

*Example IV*

|    |                    |     |
|----|--------------------|-----|
| 50 | Polyvinyl chloride | 100 |
|    | Plasticiser        | 500 |
|    | Ester gum          | 3   |
|    | Burnt sienna       | 4   |

**55** A much softer composition with reasonable surface tack suitable for low speed rollers.

*Example V*

|                    |     |
|--------------------|-----|
| Polyvinyl chloride | 100 |
| Plasticiser        | 20  |
| Modified phenolics | 5   |

A much harder composition with good surface tack ideal for high speed rollers.

*Example VI*

|                    |     |
|--------------------|-----|
| Polyvinyl chloride | 100 |
| Plasticiser        | 400 |
| Ester gum          | 5   |

A very soft substance suitable for low speed rollers.

*Example VII*

|             |     |
|-------------|-----|
| Plastic     | 100 |
| Plasticiser | 300 |
| Ester gum   | 100 |

An extremely tacky soft surface unsuitable for rollers but suitable for special purposes where high tackiness is desirable.

*Example VIII*

|                    |     |
|--------------------|-----|
| Polyvinyl chloride | 100 |
| Plasticiser        | 300 |
| Resin              | 20  |

A soft substance with good tack suitable for low speed rollers.

Although an plasticisers which are compatible with the thermo-plastic and the phenolics and resins are suitable, the following have proved particularly suitable for use with vinyl chloride resin: tri-octyl phosphate; di-octyl phthalate; di-ethylene glycol; di-ethylene glycol mono-ethyl ether; and di-ethylene glycol di-butyl ether. These have been found particularly suitable for use with ester gum as a tackifier but may be used with any resin which is compatible with nitrocellulose or polyvinyl chloride and the above mentioned group of plasticisers. Such resins are those generally found in the ester gum class utilized as varnish or lacquer resins. With regard to compatibility of plasticisers, it is merely necessary to test the resin with a small amount of plasticiser to determine whether or not the two may be used in the same roller.

Accordingly, it will be seen that this invention permits a wide application in the printing roller

and plate industry fulfilling the long felt want of providing a roller which will remain efficient at higher temperatures than are encountered in high-speed rollers and which will, in addition, efficiently print inks which contain a water base.

Various modifications and changes may be made in the preparations of the ingredients used depending upon the particular purpose to which a particular roller is to be put. Accordingly, it is not desired that the breadth of the invention be limited in any way except as set out in the accompanying claims.

What I claim as my invention is:

1. A printing roller having a core and a fixed surround on the surface whereof is formed a cylindrical inking surface coaxial to said core, said surround being composed of a homogeneous composition consisting essentially of rubbery plasticised polyvinyl chloride containing from about 1 to about 5% by weight of compatible ester gum.

2. A printing roller as defined in claim 1, in which the polyvinyl chloride is plasticised with di-octyl phthalate.

3. A printing roller as defined in claim 2, in which the proportion of di-octyl phthalate to polyvinyl chloride is substantially 13:10.

JAMES SPENCER.

## REFERENCES CITED

The following references are of record in the file of this patent:

## UNITED STATES PATENTS

| Number    | Name           | Date          |
|-----------|----------------|---------------|
| 830,432   | Hennessey      | Sept. 4, 1906 |
| 1,870,661 | Vogt           | Aug. 9, 1932  |
| 1,929,453 | Semon          | Oct. 10, 1933 |
| 2,028,712 | Swan et al.    | Jan. 21, 1936 |
| 2,075,106 | Fordyce et al. | Mar. 30, 1937 |

## OTHER REFERENCES

Fritz et al., page 41, India Rubber World, Mar. 1, 1938.

Koro seal Handbook of Tech. Info. pp. 9-12, pub. 1942 by B. F. Goodrich Co.

Koro seal Handbook of Technical Information, pages 5, 14, 15 and 19, pub. 1942 by B. F. Goodrich Co.